

# United States Patent

[19]

Newman et al.

[11] 3,762,889

[45] Oct. 2, 1973

[54] **DETERGENT MOTOR FUEL CONTAINING THE SALT REACTION PRODUCT OF A PARAFFINIC OIL OXIDATE AND A SUBSTITUTED UREA**

[75] Inventors: **Stanley R. Newman, Fishkill; Roy I. Yamamoto; Ronald W. Von Allmen,** both of Wappingers Falls, all of N.Y.

[73] Assignee: **Texaco Inc., New York, N.Y.**

[22] Filed: **Nov. 6, 1970**

[21] Appl. No.: **87,600**

[52] U.S. Cl. .... **44/66, 44/71**

[51] Int. Cl. .... **C10I 1/18, C10I 1/22**

[58] Field of Search..... **44/66, 71; 260/404.5**

[56] **References Cited**

**UNITED STATES PATENTS**

2,839,372 6/1958 Lindstrom et al. .... **44/66**

3,565,592 2/1971 Mehmedbasich ..... **44/71 X**

*Primary Examiner*—Daniel E. Wyman

*Assistant Examiner*—W. J. Shine

*Attorney*—Thomas H. Whaley and Carl G. Reis

[57] **ABSTRACT**

Salt reaction product of a paraffinic oil oxide having a Neutralization Number from 55 to 80 and a Saponification Number from 100 to 200 and a substituted urea represented by the formula:



in which  $x$  has a value from 2 to 4 and R and R' are hydrocarbyl radicals having from eight to 20 carbons, and a detergent motor fuel composition containing same.

**6 Claims, No Drawings**

**DETERGENT MOTOR FUEL CONTAINING THE  
SALT REACTION PRODUCT OF A PARAFFINIC  
OIL OXIDATE AND A SUBSTITUTED UREA**

**BACKGROUND OF THE INVENTION**

**1. Field of the Invention**

Modern internal combustion engine design and motor fuel compositions are undergoing important and substantial changes to meet new strict anti-pollution standards for exhaust gas emissions. A major change in engine design recently adopted is the feeding of blow-by gases from the crankcase zone of the engine into the intake air supply to the carburetor rather than venting these gases to the atmosphere as in the past. The blow-by gases contain substantial amounts of deposit-forming substances and are known to form deposits in and around the throttle plate area of the carburetor. These deposits restrict the flow of air through the carburetor at idle and at low speeds so that an overrich fuel mixture results. This condition produces rough engine idling, stalling and also results in excessive hydrocarbon exhaust emission to the atmosphere.

Motor fuel compositions are undergoing substantial changes. The partial or complete removal of tetraalkyl lead compounds from gasoline is well under way and is bringing about a complete reformulation of the base fuel composition and the octane levels of same. The new fuel composition will require a highly effective detergent additive in order to satisfy the strict anti-pollution standards.

**2. Description of the Prior Art**

Numerous patents have issued disclosing the use of urea derivatives to effect improvements in gasoline compositions. U.S. Pat. No. 2,373,372 discloses alkylated and arylated ureas for improving the anti-knock value of gasoline. U.S. Pat. No. 2,683,081 discloses N-hydrocarbyl-N'-hydroxyphenyl ureas as anti-oxidants for gasoline. U.S. Pat. No. 2,772,148 discloses N-alkyl-N',N'-di(carboxymethyl) urea as a rust inhibitor for hydrocarbon fuels. U.S. Pat. No. 2,965,458 discloses ester-type and acid type petroleum hydrocarbon oxides and U.S. Pat. No. 3,615,294 discloses a detergent motor fuel composition containing substituted ureas.

**SUMMARY OF THE INVENTION**

A novel class of salt reaction products of a paraffinic oil oxidate and a substituted urea are provided which are useful as carburetor detergents when employed in a liquid hydrocarbonaceous fuel for an internal combustion engine. The salt reaction product comprising a specific paraffinic oil oxidate and the below described substituted urea appears to be unique in its detergency properties.

The fuel composition of the invention mitigates or overcomes the problem of deposits laydown in the carburetor of an internal combustion engine. When a gasoline of the invention is employed in a carburetor which has a substantial build-up of deposits from prior operations, a severe test of the detergency property of the fuel, this gasoline is very effective for removing substantial amounts of these preformed deposits. These properties of the gasoline contribute substantially to improved fuel combustion and cleaner exhaust and emissions to meet prevailing and planned anti-pollution goals.

**DESCRIPTION OF THE PREFERRED  
EMBODIMENTS**

The liquid paraffinic oil oxidate employed to form the salt reaction product has a Neutralization Number between 55 and 80 and a Saponification Number between 100 and 200. Preferably, this paraffinic oil oxidate has a Neutralization Number between 60 and 80, a Saponification Number between 120 and 165, an unsaponifiable content less than about 55 percent and a viscosity less than 100 SUS at 210°F. The oxidate is obtained by air oxidation of a refined paraffinic base lubricating oil having a viscosity between 90 to 350 SUS at 100°F, or more, preferably between 140 to 180 SUS at 100°F. The paraffinic base lubricating oil will also have a pour point less than 5°F and an aniline point between 214° and 225°F. It is generally convenient to employ the liquid oxidate in solution, preferably in a light distillate, mineral, lubricating oil carrier. This facilitates handling and the carrier solution can provide a very suitable medium for forming the salt reaction product. This paraffinic oil oxidate is described in the above-noted U.S. Pat. No. 2,965,458.

The substituted urea component of the salt reaction product has the formula:



in which  $x$  has the value of from 2 to 4 and  $\text{R}$  and  $\text{R}'$  are hydrocarbyl radicals having from 8 to 20 carbon atoms each. In a preferred embodiment  $x$  has a value of 3, and  $\text{R}$  and  $\text{R}'$  each represent a saturated secondary aliphatic radical having from 10 to 15 carbon atoms.

The salt reaction product of the invention is prepared by reacting the prescribed paraffinic oil oxidate with the prescribed hydrocarbon substituted urea. In general, suitable proportions of the reactants are employed so that a substantial proportion and preferably all of the acid reacting groups in the paraffinic oil mixture oxidate are reacted to form salt reaction products. The specific proportion of urea to oxidate is determined by their total Base Number and total Acid Number, respectively. This reaction can be conducted at normal room temperature or at any elevated temperature below the decomposition temperature of either reactant or the reactant mixture. It is preferred to conduct this reaction at a temperature ranging from about 60° to 90°C but below 100°C where amide formation may occur. No further purification of the product is required.

Any gasoline suitable for a spark-ignited, internal combustion engine can be used in the practice of this invention. In general, the base fuel will consist of a mixture of hydrocarbons in the gasoline boiling range, i.e. from about 75° to 450°F. The hydrocarbon components can consist of paraffinic, naphthenic, aromatic and olefinic hydrocarbons obtained by thermal or catalytic cracking or reforming of petroleum hydrocarbons. This base fuel will generally have a Research Octane Number above 85 and preferably above 90.

The salt reaction product of the invention can be advantageously employed in the motor fuel at a concentration ranging from about 0.005 to 0.05 weight percent. The preferred concentration of the additive is from about 0.01 to 0.03 weight percent.

The following examples illustrate the preparation of the salt reaction product of the invention.

#### EXAMPLE I

180 g (0.60 mole) of N-cocopropylene diamine (commercial Duomeen C) was placed in a 500 ml flask equipped with a thermometer, condenser, magnetic stirrer and a sintered glass tube. 18g (0.30 mole) of urea was added and the mixture heated for three hours at 160°C. A slow steady nitrogen flow was maintained to sweep out ammonia being evolved. The nitrogen flow was continued until the reaction product returned to room temperature. The reaction product was diluted with approximately 600 ml of a 50/50 ether/benzene mixture and washed alternately with 6 × 100 ml of 1.5 N hydrochloric acid. After washing with 6 × 100 ml of 10 percent sodium carbonate, the product was washed with water until the wash was slightly basic, i.e., less than pH 8. The product was dried over  $\text{CaSO}_4$  and  $\text{Na}_2\text{SO}_4$ , filtered and the solvent removed by vacuum distillation at 0.5mm Hg over a steam bath.

The N-cocopropylenediamine-urea derivative, also known as 3,3'di(cocamino) di-n-propylurea, had a total Base Number (ASTM D-664) of 167 (Theory 178) and a nitrogen content of 9.3 percent (Theory 8.9). Duomeen C is an Armour Company having the formula:



where R is an alkyl radical derived from coconut fatty acids.

A paraffinic mineral oil distillate was oxidized by air blowing as described in U.S. Pat. No. 2,965,458 to produce a liquid oxidate product having an SUS viscosity at 210°F of about 82.2, a Neutralization No. of about 73.4 and a Saponification Number of about 137. The foregoing product was dissolved in a mineral oil having a viscosity of 100 SUS at 100°F. The resultant solution was filtered and referred to as an oxidate concentrate consisting of about 25 (weight) percent of liquid oxidate in the solution. This concentrate had a TAN (Total Acid Number) of 12.7.

5 grams of the 3,3' di(cocoamine)-di-n-propylurea and 66 grams of the above oxidate were mixed at room temperature and permitted to react overnight. The resultant solution containing the salt reaction product in an oil solution was suitable as a motor fuel additive.

#### EXAMPLE II

5 grams of 3,3'-di(oleylamino)di-n-propylurea having a TBN of 130 were mixed with 51 grams of the oxidate concentrate of Example I and reacted overnight at room temperature to form an oil solution of the salt reaction product.

#### EXAMPLE III

5 grams of 3,3'-di( $\text{C}_{15}$  sec. alkylamino)di-n-propylurea having a TBN of 140 and 55 grams of the oxidate concentrate of Example I were mixed and reacted overnight at room temperature to form an oil solution of the salt reaction product.

#### EXAMPLE IV

5 grams of 3,3'-di( $\text{C}_{11}$  sec. alkylamino)di-n-propylurea having a TBN of 178 and 70 grams of the oxidate concentrate of Example I were reacted at room temperature for about 8 hours to form an oil solution of the salt reaction product.

#### EXAMPLE V

10 5 grams of 3,3'di( $\text{C}_{10}-\text{C}_{14}$  sec. alkylamino)di-n-propylurea having a TBN of 205 and 80 grams of the oxidate concentrate of Example I were reacted at room temperature for about 8 hours to form an oil solution of the active salt reaction product.

15 The salt reaction product of the invention was tested for its effectiveness as a carburetor detergent additive for gasoline in the Chevrolet V-8 Carburetor Detergency Test. This test is run on a Chevrolet V-8 engine mounted on a test stand using a modified four barrel carburetor. The two secondary barrels of the carburetor are sealed and the fuel feed to each of the primary barrels is arranged so that an additive fuel can be run in one barrel and a base fuel run in the other. The primary carburetor barrels were also modified so that they had removable aluminum inserts in the throttle plate area in order that deposits formed on the inserts in this area could be conveniently weighed.

20 30 In the procedure designed to determine the effectiveness of an additive fuel to remove preformed deposits in the carburetor, the engine is run for a period of time usually 24 or 48 hours using the base fuel as the feed to both barrels with engine blow-by circulated to the air

25 35 inlet of the carburetor. The weight of the deposits on both sleeves is determined and recorded. The engine is then cycled for 24 additional hours with base fuel being fed to one barrel, additive fuel to the other and no blow-by to the carburetor air inlet. The inserts are then removed from the carburetor and weighed to determine the difference between the performance of the additive and non-additive fuels in removing the preformed deposits. After the aluminum inserts are cleaned, they are replaced in the carburetor and the

40 45 process repeated with the fuels reversed in the carburetor barrels to minimize differences in fuel distribution and barrel construction. The deposit weights in the two runs are averaged and the effectiveness of the base fuel and of the additive fuel for removing deposits expressed in percent.

50 55 The base fuel employed in the following examples was a premium grade gasoline having a Research Octane Number of 101 and contained 3 ml of tetraethyl lead per gallon. This gasoline consisted of about 25.5 percent aromatic hydrocarbons, 20 percent olefinic hydrocarbons and 54.5 percent paraffinic hydrocarbons and boiled in the range from about 89°F to 362°F.

60 65 The carburetor detergency test results obtained from the base fuel containing the salt reaction products described above are set forth in the following Table. The additive-containing fuels contained 5 PTB (pounds per one thousand barrels of fuel) of the urea and enough of the oxidate as a solution in mineral oil to completely neutralize the urea.

TABLE I  
Chevrolet Carburetor Detergency Test Deposit Removal

| Run | Fuel                         | Deposit Build-up<br>mg* | Deposit Removed<br>mg | % Effective | % Removal |
|-----|------------------------------|-------------------------|-----------------------|-------------|-----------|
| 1   | Base Fuel                    | 25.6                    | 0.7                   | 3           |           |
| 2   | Base + 71 PTB<br>Example I   | 26.6                    | 13.6                  | 51          | 48        |
| 3   | Base Fuel                    | 25.6                    | 1.0                   | 4           |           |
| 4   | Base + 56 PTB<br>Example II  | 29.2                    | 17.9                  | 61          | 57        |
| 5   | Base Fuel                    | 25.8                    | 6.2                   | 24          | 10        |
| 6   | Base + 60 PTB<br>Example III | 25.9                    | 14.7                  | 57          | 33        |
| 7   | Base Fuel                    | 22.0                    | -1.1**                | -5          |           |
| 8   | Base +75 PTB<br>Example IV   | 21.2                    | 16.7                  | 79          | 84        |
| 9   | Base Fuel                    | 19.5                    | -3.6                  | -18         | 15        |
| 10  | Base + 85 PTB<br>Example V   | 20.4                    | 13.6                  | 67          | 85        |

\*Built up with base fuel

\*\* Additional deposits formed

In the foregoing tests, Runs 2, 4, 6, 8 and 10 show that the salt reaction product of the invention provides an outstanding improvement in the carburetor detergent properties of the additive-containing gasoline as compared to the base fuel.

The motor fuel composition of the invention can contain any of the additives normally used in gasoline including corrosion inhibitors, anti-oxidants, anti-icing compounds and tetraalkyl lead anti-knock mixtures.

We claim:

1. A motor fuel composition comprising a mixture of

hydrocarbons in the gasoline boiling range containing a minor carburetor detergent amount of the neutral salt reaction product formed at a temperature from 60 to 90°C. of a substituted urea represented by the formula:



in which x has a value from 2 to 4 and R and R' are hydrocarbyl radicals having from eight to 20 carbon atoms and a paraffinic oil oxidate having a Neutralization Number from 55 to 80 and a Saponification Number from 100 to 200.

2. A motor fuel composition according to claim 1 containing from about 0.005 to 0.05 weight percent of said salt reaction product.

3. A motor fuel according to claim 1 in which said substituted urea is 3,3'-di(oleylamino)-di-n-propylurea.

4. A motor fuel composition according to claim 1 in which x has a value of 3 and R and R' are aliphatic hydrocarbon radicals having from 10 - 15 carbon atoms.

5. A motor fuel composition according to claim 1 in which said substituted urea is 3,3'-di(cocoamino)di-n-propylurea.

6. A motor fuel composition according to claim 1 in which said substituted urea is 3,3'-di-(C<sub>10</sub>-C<sub>14</sub> sec. alkylamino)-di-n-propylurea.

\* \* \* \* \*

35

40

45

50

55

60

65